# EUROPEAN PATENT SPECIFICATION

(11) **EP 0 056 704 B1**
(45) Date of publication and mention of the grant of the patent: **20.08.1986**
(21) Application number: 82300160.7
(22) Date of filing: 12.01.1982
(51) Int. Cl.: B05D 1/26, B05D 1/34, B05D 5/06, B05C 5/02, B05C 9/06

(54) **Coating apparatus and process**
Vorrichtung und Verfahren zum Aufbringen eines Überzuges
Dispositif et procédé pour appliquer un enduit

(30) Priority: 21.01.1981 US 226697; 21.01.1981 US 226699; 21.01.1981 US 226705
(43) Date of publication of application: 28.07.1982
(73) Proprietor: ALCAN INTERNATIONAL LIMITED, Montreal Quebec H3A 3G2 (CA)
(72) Inventor: Wollam, Carl A., Cortland Ohio (US); Gailey, J. Lynn, Newton Falls Ohio (US); Chalmers, Alexander A., Warren Ohio (US)
(74) Representative: Brooke-Smith, Fred

## Description

This invention relates to coating processes and apparatus, and in particular to processes and apparatus for coating surfaces of strip articles of indeterminate length.

In coating operations as herein contemplated, an initially wet, flowable coating material is applied to a surface of a substrate that is at least substantially impervious thereto, for covering the substrate surface with a continuous adherent coating layer. One especially important application of the invention, to which detailed reference will be made for purposes of illustration, is the coating of metal strip with a protective and/or decorative layer of paint or the like, prior to cutting orforming of the strip into shingles, siding or soffit panels, building trim members, or other products.

Metal strip (i.e. strips of sheet metal of indeterminate length, usually stored as coils) is continuously coated, in commercial practice, by advancing the strip longitudinally past a locality where a wet coating material such as paint is applied to one or both major surfaces of the strip, and then through a zone where the coating is cured or dried with heat. Known techniques for applying wet coating material to a strip surface including spraying, transfer from rolls, and deposit of the coating material on the strip surface immediately ahead of a doctor blade or dam which has the purpose of establishing a desired coating thickness. In the latter instance, the blade or dam, as will be understood, has a thin edge extending transversely across and very slightly spaced from the surface to be coated; the deposited wet coating material puddles on the upstream side of the blade or dam and is carried thereunder in a thin layer on the moving surface.

While coating operations using a blade or dam are advantageous from the standpoint of mechanical simplicity, they (like other coating techniques, e.g. spray and roll-coating) do not afford assured or easily attainable high uniformity of coating thickness, especially in the coating of metal strip which commonly has wavy edges, an "oil-canned" central area, or other slight deformations tending to cause variation in the effective spacing between the blade or dam edge and the strip surface and consequently in the thickness of the coating layer determined by that spacing. In order to achieve an adequate coating thickness at all points on the strip surface, therefore, it is commonly necessary to apply a coating layer having a greater average thickness (and thus to consume more coating material) than would be required if the thickness could be made more uniform. This consumption of excess coating material is economically undesirable.

An additional disadvantage of such conventional coating arrangements is the waste of coating material that occurs, e.g. through overflow, owing inter alia to shortcomings in the effectiveness of the metering action provided by these arrangements. Moreover, there is a tendency for air to be picked up in the coating material ahead of the doctor blade, and to become entrapped in the coating, especially at fast coating speeds.

Further complications are encountered when it is attempted by conventional means to provide a coating layer having a striped, streaked, marb- leized or otherwise variegated pattern. It has been proposed (in U.S. Patent No. 3106480) to supply paint of different colours to different locations along a common reservoir defined in the nip between two rolls, one of which transfers the paint from the reservoir to a sheet surface to be coated; but in use of blade or dam-type coating arrangements (which, as noted, offer the important advantage of mechanical simplicity) it has heretofore been considered necessary to provide separators for isolating the different colours in the coating material pool or puddle upstream of the dam, as shown for example in U.S. Patents No. 2695005 and No. 3883898. Such separators add to the structural complexity of the coating apparatus and prevent or at least greatly restrict the provision of controlled variation in the colour patterns produced.

European Specification No. 3970 discloses a coating apparatus of the type indicated on the prior art portion of claim 1. In this known apparatus a strip form article to be coated on one surface is moved about the periphery of a rigid roller, the outer surface of the strip having facing it a diaphragm urged towards the strip by fluid pressure. The surface to be coated is pulled through a reservoir of the coating material where the.strip enters between the roller and the diaphragm T.

According to the present invention in one aspect there is provided a process for coating a major surface of a strip article of indeterminate length, including the steps of continuously advancing the article longitudinally past a dam extending transversely of said major surface in adjacent spaced relation thereto while supplying a flowable liquid coating material to said major surface immediately ahead of said dam and, immediately beyond said dam, advancing said article longitudinally past a wall of extended length in the direction of strip advance and facing said major surface, said strip being uniformly restrained by restraining means against movement of said major surface away from said wall beyond a predetermined distance equal to a desired wet thickness of said coating material on said major surface characterised in that the said wall of extended length is provided by a rigid member which wall is equidistantly spaced from a rigid support constituting the restraining means, said rigid member being fixedly securable relative to the restraining means.

In another aspect the invention provides apparatus for forming a continuous adherent coating layer on a major surface of a strip article of indeterminate length comprising means defining a path of advance of said article lengthwise of itself including an extended wall facing said major surface of said article and so arranged that the advancing article moves longitudinally relative thereto and means for uniformly restraining said article against movement of said major surface away from said wall beyond a predetermined distance during advance of said article past said wall, means constituting a dam extending transversely of the path of article advance so as to be disposed in adjacent spaced relation to said major surface of the article and means for supplying a wet flowable coating material to said major surface ahead of said dam characterised in that said extended wall is constituted by a surface of a rigid member which surface is equidistantly spaced from a rigid support constituting the said restraining means and in that means are provided for fixedly securing said rigid member relative to said restraining means.

The means-for thus restraining the strip may, for example, comprise a second wall spaced uniformly from the first-mentioned wall so as to define therewith a gap (through which the strip advances) equal in width to the sum of the strip thickness and the desired coating thickness.

This feature of advancing the strip past a wall of extended length, immediately beyond the dam, while uniformly restraining the strip against movement away from the wall beyond a predetermined distance, is found to produce an advantageously high uniformity of coating thickness even on strip which may be wavy-edged, oil-canned, or otherwise deformed. As at present believed, the applied wet coating material, lying under pressure between one surface of the strip and the facing wall (relative to which the strip is moving), forces the strip away from the wall bv a hvdroplaning action, thereby (i.e. since the strip is uniformly restrained against such movement beyond a predetermined distance) smoothing out the strip deformations for the duration of advance of the strip past the wall so as to achieve substantial uniformity of spacing between all points on the coated strip surface and the facing wall. The latter spacing determines the wet thickness of the coating; hence the coating on the strip is of desirably uniform thickness, notwithstanding that the strip deformations reappear as the strip emerges beyond the wall. Better metering of the coating material can be obtained in use of the invention than in conventional techniques using rolls or doctor blades; substantially all the supplied coating material is usefully consumed to provide the desired coating, with virtually no loss due to spillage over the sides.

The downstream end of the wall facing the coated strip surface (i.e. the end remote from the dam in the direction of strip advance) is preferably a sharp edge providing an abrupt surface discontinuity rather than a radiussed edge which could cause cavitation problems and resultant irregularities in the produced coating. Thus, the downstream wall edge may be constituted as the intersection of the strip-facing wall surface with a surface (of the wall structure) facing downstream and lying in a plane oriented at an angle of at least about 90° to the direction of strip advance. On the other hand, it is preferred that the dam at or constituting the upstream end of the wall have a radiussed or chamfered edge for leading the coating material onto the strip surface and gradually initiating the fluid pressure which, between the wall and the strip surface, provides the above-described hydroplaning effect. It is also frequently preferable that the body or pool of liquid coating material ahead of the dam be maintained under positive pressure.

It is additionally found that the process and apparatus of the invention enable stripes and other variegated patterns of colours or shades to be achieved in the produced coating by supplying coating material of different colours or shades to different portions (spaced across the width of the strip) of a single continuous pool or puddle of the coating material extending along the inlet side of the dam, i.e. without employing any separators to isolate these different shades or colours in the pool. The nature of the patterns produced is dependent on the locations and relative quantities of the different shades or colours thus supplied, and can be controllably varied as desired during the coating of a single continuous strip surface by varying one or more of these factors. The invention in particular embodiments includes means of effecting such variation.

In apparatus in accordance with the invention, the wall facing.the coated surface of the strip may be an extended surface of a stationary plate past which the strip advances, an upstream portion of the plate being shaped to constitute the dam, although it will be understood that in a broad sense the requisite movement of the strip relative to this facing wall could be achieved by moving the wall along a stationary strip. The means for- restraining the strip against movement away from this wall may also be a wall constituted by a stationary plate. In some embodiments of the invention, however, this other wall is an endless surface moving in the same direction and at the same rate as the strip, so as to prevent abrasion.

Some embodiments ofthe invention will now be described by way of example with reference to the accompanying drawings in which:
Figure 1 is a simplified schematic perspective view illustrating the performance of the process of the present invention in an illustrative embodiment;
Figure 2 is a plan view of one embodiment of the apparatus of the invention, suitable for performing the process of Figure 1;
Figure 3 is a side elevational view of the apparatus of Figure 2;
Figure 4 is a cross-sectional elevational view taken along the line 4-4 of Figure 3;
Figure 5 is an enlarged fragmentary sectional view taken along the line 5-5 of Figure 2;
Figure 6 is a side elevational view of another embodiment of the apparatus of the invention;
Figure 7 is a fragmentary cross-sectional elevational view taken along the line 7-7 of Figure 6;
Figure 8 is a side elevational view of a further modified embodiment of the apparatus of the invention;
Figure 9 is a bottom view of the coating supply-controlling element of the apparatus of Figure 8;
Figures 10 and 11 are, respectively, cross-sectional views taken along the lines 10-10 and 11-11 of Figure 9;
Figure 12 is a plan view of another embodiment of the apparatus of the invention;
Figure 13 is a side elevational sectional view taken along the line 13-13 of Figure 12;
Figure 14 is a simplified schematic plan view of yet another embodiment of the apparatus of the invention;
Figure 15 is a side elevational sectional view taken along the line 15-15 of Figure 14;
Figure 16 is a simplified schematic side elevational view of a still further embodiment of the apparatus of the invention.
Figures 17 and 18 are plan and sectional views, respectively, of another embodiment of the invention;
Figure 19 is a schematic side elevation view of a coating line incorporating the embodiment of Figures 17 and 18;
Figure 20 is a simplified schematic perspective view of another embodiment of the invention;
Figure 21 is a schematic side elevational sectional view of another illustrative embodiment of the apparatus of the invention;
Figure 22 is a plan view taken as along the line 22-22 of Figure 21;
Figure 23 is a transverse elevational sectional view taken as along the line 23-23 of Figure 21;
Figure 24 is a schematic plan view, similar to Figure 22 of another embodiment of the invention;
Figure 25 is a transverse elevational sectional view taken along the line 25-25 of Figure 24;
Figure 26 is an enlarged fragmentary detail sectional view of a portion of the disc of the apparatus of Figure 24, taken as along the line 26-26 of Figure 24;
Figure 27 is a similarly enlarged fragmentary detail sectional view taken as along the line 27-27 of Figure 26;
Figure 28 is a diagrammatic plan view illustrating the effect, on the produced coating patterns, of angular displacement of the disc in the apparatus of Figure 24;
Figure 29 is a plan view of a further embodiment of the apparatus of the invention;
Figure 30 is an enlarged side elevational view, partly in section, taken along the line 30-30 of Figure 29;
Figure 31 is an enlarged bottom plan view of the disc of the apparatus of Figure 29;
Figure 32 is a further enlarged sectional view of the disc, taken along the line 32-32 of Figure 31; and
Figure 33 is a similarly enlarged, fragmentary sectional view of the disc, taken along the line 33-33 of Figure 31.

Referring first to Figure 1, the invention will be described as embodied in a process for continuously coating one major surface 10 of a metal (e.g. aluminium) strip 11 of indeterminate length with a continuous layer 12 of an initially wet coating material, such as paint, extending over the entire strip surface. For such coating, the strip is continuously advanced longitudinally (as from a supply coil 14) along a defined path past a locality 15 at which the wet paint is applied to the surface 10, and thence to a heating zone (not shown) where the coating is cured or dried. The other major surface 16 of the strip can be coated before or after the described coating of the surface 10, or left uncoated. Once the coating of the strip is complete, it can be formed and cut into a desired product such as siding panels.

The apparatus with which the process of the invention is performed is shown (by way of example) in Figure 1 as comprising a pair of rigid flat plates 18 and 20 fixedly mounted, in superposed facing uniformly spaced relation to each other, at a portion of the path of advance of the strip 11 at which the strip major surfaces are substantially horizontal with surface 10 facing upwardly, the plates 18 and 20 being respectively disposed above and below the strip so that the path of strip advance passes between them. The upper plate 18 has an elongate reservoir cavity or trench 22 dimensioned to extend across the full width of the strip 11 and opening downwardly toward the upper surface 10, for confining a body or pool of liquid coating material such as paint in contact with the strip surface 10. Paint is supplied to the cavity or trench 22 through a plurality of passages 24 opening downwardly through the upper surface of the plate 18 into the cavity at locations spaced along the length thereof, i.e. across the width of the strip 11. Immediately beyond the cavity 22, the plate has a smooth, downwardly facing horizontal planar surface 26 that extends across the full width of the strip and also extends downstream from the cavity for a substantial distance in the direction of strip advance; the lower plate 20 has a smooth upwardly-facing horizontal planar surface 28 also extending across the full width of the strip and longitudinally of the strip over at least the full extent of the upper plate surface 26.

The surfaces 26 and 28 respectively constitute the upper and lower walls of a gap 30 of extended length in the direction of strip advance. Since these surfaces 26 and 28 lie in parallel horizontal planes (and are thus spaced apart by a uniform distance at all points) the gap 30 is of uniform height. The spacing between the two plate surfaces (i.e. the height of gap 30) is selected to be equal to the thickness of the strip 11 plus a desired wet thickness of coating layer on the strip surface 10, and is maintained at a fixed value during any given coating operation, although the spacing between the plates may be adjustable. The internal surface 32 of the upper plate 18 which defines the downstream side of the reservoir cavity 22 constitutes a dam, extending transversely across the strip surface 10 at the inlet end of the gap 30 and retaining the coating material on its upstream side in the reservoir.

In the practice of the present process, the locality 15 at which the coating material is applied to the strip surface 10 is the location of the reservoir cavity 22. As the strip advances past the cavity, the surface 10 is progressively brought into contact with the pool of wet flowable coating material therein, across its full width. The advancing movement of the strip draws coating material from the cavity on the strip surface 10 into the gap 30, i.e. into the space between the strip surface 10 and the facing gap wall 26, filling that space and forcing the strip against the other gap wall 28 notwithstanding any undulating or other deformation initially present in the strip. In this way, as the strip advances through the gap, the distance from the strip surface 10 to the gap wall 26 becomes uniform at all points and, since the space therebetween is filled with flowable coating material, a uniform wet thickness of coating layer over the entire surface 10 is achieved, even though as the strip emerges from the gap at the outlet or downstream end thereof any deformation initially present in the strip reappears. Thus, with progressive supply of wet coating material to cavity 22 (by gravity feed, in the embodiment shown) at a rate sufficient to maintain the gap 30 completely filled, the strip surface 10 is uniformly and continuously coated.

When paint of a single colour is supplied to the cavity 22 through all the passages 24, a single-colour coating is produced. Striped or other desired pattern effects can be achieved by supplying paint of different colours or shades through the different passages. For example, if the passages 24 are respectively located at the centrelines of longitudinal zones of equal width on the strip surface, and are all supplied with equal volumes of paint per unit time (in respectively different colours 1, 2 and 3), the produced coating will be constituted of well-defined .parallel stripes 36a, 36b, 36c of the different colours without significant blurring or blending between stripes, even though the cavity 22 is a single, continuous, undivided reservoir. The stripes can be varied in relative width during the coating operation, and blended effects can be achieved by varying the relative rates of feed of paint to the different passages. Thereby controllably varied colour patterns of longitudinal stripes of striations can readily and conveniently be produced on the coated surface.

The structure of the coating apparatus of Figure 1 is illustrated in further detail in Figures 2 to 5. As there shown, the coating cavity 22 is machined across the width of the upper plate 18 and is provided with end plugs 40 for laterally enclosing the cavity to confine the liquid coating material therein. The plates 18 and 20 are secured together by means of bolts 42 respectively located at each corner of the plates. Each bolt 42 is inserted downwardly through a hole in the top plate 18 and is threaded into the bottom plate 20; a helical spring 43 is disposed in surrounding relation to the shank of each bolt 42 between the plates and is under compression between the plates 18 and 20. The bolts and springs serve to maintain the facing surfaces 26, 28 of the two plates (which, in this embodiment, are both highly polished planar surfaces) uniformly spaced apart over the full lateral and longitudinal extent of the gap 30, and to maintain the spacing fixed during any given coating operation while permitting adjustment of the spacing (for selection of a desired coating thickness) before the coating operation has begun. As a further aid in positionally stabilizing the plates, bars 45 are bolted to both sides of the bottom plate 20 and project upwardly therefrom along the sides of the plate 18 to prevent relative lateral displacement of the plates.

As best seen in Figures 3 and 5, in this embodiment of the apparatus the horizontal planar surface 28 of the lower plate 20 extends for some distance upstream of the coating cavity 22 and faces a horizontal planar surface portion 26a of the upper plate 18 ahead of cavity 22. The spacing between the upstream portion of surface 28 and the surface 26a of plate 18 is equal to the spacing between surfaces 26 and 28; i.e. the surface 26a together with the portion of surface 28 subjacent thereto cooperatively define a gap 30a equal in height to gap 30 and having an extended length along the path of strip advance.

In an illustrative example of-apparatus of the type shown in Figures 2 to 5, the width of the , surfaces 26, 28 and 28a is between 20.0 to 20.4 cm for coating strip less than 20.0 cm wide, and the length of surface 26 (which, with surface 28, defines gap 30) is slightly less than 22.9 cm in the direction of strip travel. The length of surface 26a, which, with the subjacent upstream portion of surface 28, defines the gap 30a, is about 2.9 cm along the path of strip travel. With apparatus having these dimensions, it is found that both gaps 30 and 30a are of sufficiently extended length to provide the advantageous results of the invention with respect to uniformity of coating thickness and attainment of desired striped or other pattern effects; i.e. when the direction of . strip travel is reversed from that indicated by arrow 46 in Figure 3, so that the gap 30a rather than the gap 30 is traversed by the strip after application of coating to its surface in the cavity 22, the gap 30a is found to be of sufficiently extended length in the direction of strip advance to substantial achieve the beneficial results of uniformity of coating thickness and production of desired pattern effects. In this reversely directed operation, of course, the surface 32a of the cavity 22 (opposite the previously described surface) functions as the dam.

As shown, the dam surface 32 is radiussed to lead the liquid coating material into the strip and to provide, as the strip advances past the dam, progressive development of the fluid pressure which causes hydroplaning action (forcing the strip uniformly against the plate 20) within the gap between the plates; alternatively, the surface 32 may be chamfered. It will be understood that this embodiment, the surface 26 of the plate 18 constitutes the wall facing the coated strip surface, and the plate 20 consitutes the means for uniformly restraining the strip against movement more than a predetermined distance away from that wall. The downstream end of the latter wall is a sharp edge 47 (Figure 3) formed by the intersection of surface 26 with a planar plate end surface 47a, shown as perpendicular to the direction of strip advance; more generally, the angle between the plane of surface 47a and the direction of strip advance is at least sufficient to avoid cavitation effects that could cause irregularities in the coating emerging from the gap 30. Of course, if such irregularities are desired, for particular esthetic purpose, the downstream end of the plate 18 could be shaped to provide a radiussed edge that would produce such cavitation.

Preferably, in at least many instances (and especially for application of plural colours in parallel longitudinal bands), in operation the reservoir cavity 22 is kept completely filled with paint, under pressure, at a rate corresponding to the rate of withdrawal of paint from the cavity on the coated strip surface. In this way there can be no entrapment of air in the produced coating.

It is also preferred, and at present considered advantageous for attainment of satisfactory coatings, that the strip surface to be coated be primed, i.e. with a primer coat applied prior to the coating operation.

The embodiments of the apparatus of the invention illustrated in Figures 6 to 15 incorporate various arrangements for creating desired pattern effects of different shapes of colours in the produced coatings.

In Figure 6, the illustrated apparatus comprises a top plate 50 and a bottom plate 52 having facing uniformly spaced extended horizontal surfaces co-operatively defining a gap 54 of extended length in the direction of strip advance represented by arrow 56. The top and bottom plates are secured together by bolts 58, with helical springs 60 under compression surrounding their shanks, for maintaining the desired spacing between the plates while permitting adjustment of that spacing.

The top plate 50 is formed in two pieces 50a and 50b which cooperatively define and upwardly opening coating cavity or reservoir 62 extending transversely of the path of strip advance across the full width of the strip. This coating cavity also opens downwardly onto the strip upper surface, through a relatively narrow opening 64 defined between the two top plate pieces 50a and 50b; the opening 64, which may, for example, be about 3 mm wide, likewise extends across the full width of the strip surface to be coated so as to permit liquid coating material from the cavity 62 to flow downwardly into contact with the strip surface. The generally vertical transverse surface 66 of plate portion 50b, constituting the downstream side of opening 64, serves as the dam for the coating material in this embodiment.

As a particular feature of the embodiment of Figures 6 and 7, a dividing member 68 extends across the cavity 62 and projects downwardly into the opening 64, for separating the cavity into two sections or chambers both extending across the full width of the path of strip advance and respectively located upstream and downstream of the opening 64. Member 68 is suspended from a rod 70 journalled in bearings 72 for rotation about an axis above and parallel to the long dimension of opening 64, i.e. to effect movement of the member 68 in the directions indicated by arrow 74.

In the operation of the apparatus of Figures 6 and 7, the two chambers into which cavity 62 is divided by member 68 can be respectively filled with paint of different colours. As a strip is continuously advanced through the apparatus, i.e. past the dam 66 and through the gap 54 downstream of the dam, the colour of coating material delivered from cavity 62 to the strip surface can be varied by pivotal movement of the member 68 so as to produce a coating characterized by transverse bands of different shades or colours. For example, if one of the chambers of cavity 62 contains blue paint and the other contains yellow paint, pivotal movement of the member 68 can alternately admit yellow and blue paints to the opening 64 for delivery onto the strip surface, producing alternating yellow and blue bands extending transversely of the long dimension of the strip being coated; and if the member 68 is moved to an intermediate position, both yellow and blue paints can be delivered to the strip surface at the opening 64, for blending (as the strip passes through gap 54) to produce a green band.

In the embodiment shown in Figures 8 to 11, wherein some structural features have been omitted for simplicity of illustration, the same plates 50 and 52 cooperatively defining a gap 54 and providing coating cavity 62 with a central downward opening 64 and dam surface 66 and all arranged as described above with reference to Figures 6 and 7. The direction of strip travel again is as indicated by arrow 56. In place of the member 68, however, the embodiment of Figures 8 to 11 employs a slidable supply-controlling element 76 which (like the member 68) of Figures 6 and 7.) divides the cavity 62 into two chambers and controls the delivery of liquid coating material from one or the other or both of these chambers to the surface of the advancing strip through opening 64. More particularly, member 76 includes a vertical portion 78 which serves to divide the cavity into the two chambers and a flat base portion 80 overlying the floor of the cavity 62. The base portion 80 has two parallel elongate slots 82 and 84 formed therein and separated by a median portion 86, slots 82 and 84 each being coextensive in length with the opening 64: Sliding movement of the element 76 in the directions represented by arrow 88 (Figure 8) effects variation in the supply of liquid coating material from the two chambers to the opening 64. As particularly shown in Figures 10 and 11, the lower surface of the median portion 86 is bevelled in different directions along different parts of its length to facilitate this control of colour delivery.

In the embodiment of Figures 12 and 13, the top plate 50 and bottom plate 52 cooperatively defining a gap 54 of uniform height and extended length in the direction 56 of strip advance are generally similar in arrangement to the plates 50 and 52 of the embodiments of Figures 6 to 11. The upper plate 50, formed in two parts, defines a coating cavity 62 communicating downwardly through an opening 64 with the surface of the strip to be coated, the downstream edge 66 of opening 64 constituting a dam.

In the embodiment of Figures 12 and 13, however, the cavity 62 is divided into upstream and downstream chambers by a thin spring steel member 90 which projects downwardly into the opening 64. At each of plural (e.g. six) locations across the width of the path of strip advance, there are provided in the upper plate 50 pairs of opposed small air cylinders 92 for locally controlling the position of the spring steel divider 90. As illustrated, the pistons of each pair of the cylinders 92 project toward each other and abut the divider 90 in opposed relation so that by operation of the cylinders the divider 90 can be flexed to admit paint from either one of the other of the two coating cavity chambers into the opening 64 for delivery to the strip surface. The several pairs of cylinders 92 may be operated in unison or independently, taking advantage of the flexibility of the divider 90; thus, with paint of different colours in the two chambers of cavity 62 (these two chambers being respectively supplied with paint through ports 94 and 96), paint of one colour can be delivered across the full width of the advancing strip, or alternatively paint of different colours can be delivered to different portions of the strip surface across the width thereof, by appropriate operation of the cylinders 92. i.e. flexing the divider 90 in a common direction or in a multiplicity of directions.

In the embodiment of Figures 14 and 15, there are, again, upper and lower stationary rigid plates respectively designated 100 and 102 with facing flat extended horizontal surfaces cooperatively defining a gap .104 of uniform height through which a strip to be coated advances in the direction represented by arrow 106. The upper plate in the embodiment of Figures 14 and 15 has plural reservoirs or cavities opening downwardly toward the strip surface to be coated; these include a main cavity 108 extending across the full width of the strip supplied through ports 110, and two auxiliary cavities 112 located downstream of the cavity 108. Each of the cavities 112 has its long dimension oriented at an oblique angle to the long dimension of the cavity 108 and extends across only a portion of the width of the strip surface to be coated. In addition, downstream of the cavities 112, on the downwardly facing surface of the upper plate 100 (which surface constitutes the upper wall of the gap 104), there are provided plural longitudinally oriented grooves 114 which cooperate with the cavities 112 in creating a striated appearance in the produced coating.

It will be understood that all of the embodiments shown in Figures 6 to 15 function in essentially the same manner for performance of the process of the invention. That is to day, in each case a strip to be surface coated is continuously advanced through the apparatus, between the upper and lower plates thereof, while liquid coating material is continuously deposited on the upwardly facing surface of the strip from a reservoir or cavity, the downstream side of which (extending transversely across the strip surface) constitutes a dam. Immediately beyond the dam, the strip advances between upper and lower walls of of a gap of extended length in the direction of strip advance, the strip moving relative to both walls, and the spacing between the walls being equal to the strip thickness plus a desired wet thickness of the applied coating layer.

In the embodiment illustrated in Figure 16, a rigid stationary plate.120 is disposed in adjacent relation to a rotatable drum 122 having a cylindrical outer surface 124, the drum rotation about a horizontal axis in the direction indicated by arrow 126. Plate 120 has a downwardly facing smooth rigid arcuate surface 128 disposed in proximate spaced relation to the drum surface 124. This plate surface 128 is concentric with the drum surface 124 and is of extended length in the direction 126 of drum rotation, being also at least equal in width to the surface of strip to be coated by the apparatus. The spacing between surface 128 of plate 120 and drum surface 124 is uniform throughout the entire extent of surface 128; hence the drum surface 124 and the plate surface 128 respectively constitute the lower and upper walls of a gap 130 of uniform height and extended length, through which a strip article such as roetal strip 132 continuously advances in the direction represented by arrow 134.

At the upstream or inlet extremity of the surface 128, the plate 120 has an edge portion 136 extending transversely across the path of strip advance and serving as a dam for liquid coating material which is deposited on the strip surface (by suitable means, not illustrated) ahead of the dam. The pool of liquid coating material thus deposited on the strip is laterally confined by plate portions 138.

The operation of the apparatus of Figure 16 in the performance of the process of the invention is generally similar to that of the other embodiments already described, except that as the strip advances, the drum 122 is rotated in the same direction and at the same rate as the strip, so that while the strip is advancing through the gap 130 and moving relative to the upper gap wall 128 of stationary plate 120, the lower gap wall or drum surface 124 moves with the strip. That is to say, there is no relative movement between the strip and the drum surface and therefore no abrasion such as can result if the lower gap wall is stationary. The coating material deposited on the upwardly facing surface of the strip prevents abrasion between the upper strip and the upper wall of the gap.

Figures 17 and 18 illustrate one currently preferred further embodiment of the apparatus of the invention, adapted for (though not limited to) production of a coating having a pattern of lines or striations, e.g. simulating the appearance of natural wood grain. In this embodiment, an aluminium strip 170 to be coated is advanced longitudinally by means including a back-up roll 172 over which the strip passes. A coating device 174 applies a coating layer 176 of paint to a major surface 178 of the strip at a locality at which the strip is held against the roll 172 with the surface 178 exposed and facing outwardly. This device includes a block or plate 180 mounted immediately adjacent the roll 172 at that locality and having a surface 182 curved concavely to conform to the surface of the roll and facing the roll in a position to define, with the roll surface, an arcuate gap through which the strip passes while being coated. A horizontally elongate, axially rectilinear reservoir trench 184 for confining a body of liquid coating material (paint) is formed in the end portion of the plate 180, and opens through the plate surface 182 toward the strip surface 178; thus the trench, which is oriented with its long dimension parallel to the axis of roll 172 and perpendicular to the direction of strip advance (represented by arrow 186), has an open long side, but is otherwise enclosed by a side wall (preferably generally semicylindrical) and flat end walls. The back-up roll 172 is positioned to maintain the strip surface 178 is proximate facing relation to the open long side of the trench so that the surface 178 constitutes a moving wall effectively closing the open trench side.

During a coating operation, the strip 170 is continuously advanced over the back-up roll while the trench 184 is maintained continuously entirely filled with paint, which deposits on the passing strip surface 178 as a continuous wet coating layer having a thickness determined by the spacing between the outlet side edge 188 of the trench and the strip surface 178. Beyond the trench the coating layer passes through a uniform gap, defined by a portion of the plate surface 182, of extended length in the direction of strip travel; the provision of this gap aids in assuring the smoothness and uniformity of thickness of the coating emerging from beneath the sharp outlet edge 190 of the plate 180.

Three paint-delivery apertures (respectively designated 192, 194 and 196) are formed in the side wall of the trench 184, at localities spaced apart along the length of the trench and spaced from (viz. directly opposite) the open long side of the trench. The central aperture 194 is positioned halfway between the ends of the trench; the apertures 192 and 196 are respectively positioned between the aperture 194 and the opposite ends of the trench, at distances (from aperture 194) each equal to one third of the total length of the trench, so that the three apertures are respectively centered in adjacent thirds of the length of the trench.

Each aperture constitutes the open outlet end of a main bore extending through the plate 180 and having T-junction with a transverse bore in the plate at a locality spaced from the aperture. The arrangement of main bore 198 and transverse bore 200 associated with aperture 192 is shown in Figure 8; the other two apertures, 194 and 196, have identical bore arrangements. A supply 202 of paint of a first colour, including a pump 202a and valves 202b, is connected to the main bore associated with each of the three apertures, while a supply 204 of paint of a second colour, also including a pump and valves, is connected to the transverse bore of each aperture, as represented diagrammatically in Figure 18. The main and transverse bores associated with each aperture, together with the paint supplies, cooperatively constitute means for delivering concurrent laminar flows of two liquid coating materials (two colours of paint) to the trench along a common path through that aperture.

Conveniently, for the illustrative example of operation now to be described, the two colours of paint are supplied to the device of Figures 17 and 18 at the same, substantially constant pressure, and the relative flows of the two colours at each aperture are determined by fixed orifice size, e.g. by the relative diameters of the main and transverse bores, such that a major flow of the first- colour paint and a minor flow of the second-colour paint enter the trench at each aperture. Thus, the supply 202 may include a single pump 202a but three valves 202b (downstream of the pump) for respectively separately controlling supply of the first colour paint to the three main bores 198, while the supply 204 likewise includes a single pump 204a but three valves 204b for respectively separately controlling supply of the second-colour paint to the three transverse bores 200. In a simple yet effective mode of operation, to which detailed reference will be made below, the two valves 202b and 204b associated with each aperture are electrically controlled to cause simultaneous starting or stopping of flow of both colours of paint through that aperture.

Whe the apparatus of Figures 17 and 18 is operated in this mode, with the strip 170 being continuously longitudinally advanced and the trench 184 being maintained continuously entirely filled with paint delivered at all three of the apertures 192, 194 and 196 (i.e. all of the valves 202b and 204b being open), the coating layer applied to the strip surface 178 comprises three contiguously adjacent longitudinal portions (positionally indicated by letters a, b, and c in Figure 17) respectively constituted of paint delivered at the apertures corresponding positionally to those coating portions. Thus, coating portion a is constituted of paint delivered to the trench at aperture 192; coating portion b is constituted of paint delivered at aperture 194; and coating portion c is constituted of paint delivered at aperture 196. The relative widths of coating portions a, b and c are directly proportional to the relative total flows of paint respectively delivered at the corresponding apertures. This observed result indicates that the paint delivered at each aperture fills only the portion of the length of the trench adjacent that aperture, and does not intermix with the paint being delivered to an adjacent portion of the trench through an adjacent aperture, notwithstanding that the trench is continuous and undivided along its length. Given the conditions described above, viz. that all the valves are open and that the paint of both colours is supplied at the same pressure to all apertures, the paint delivered at each aperture fills one third of the trench and the coating portions a, b and c are equal to each other in width.

Within the portion of the paint layer corresponding to each aperture, there is produced a pattern of multiple longitudinal striations of the two colours of paint delivered to the trench at that aperture in concurrent laminar flows. Thus, from the three apertures of Figure 17 there are produced three parallel patterns of longitudinal striations. It is believed that within the portion of the trench supplied through each aperture, there is established an essentially separate helical laminar flow pattern of the two colours of paint so that there are three such patterns, arranged side by side along a common axis, respectively located adjacent the three apertures in the trench of Figure 17; and it is further believed that the striated pattern results from impingement of the turns of these helical flows on the advancing strip surface.

When delivery of paint through any one of the apertures is interrupted by operation of its associated valves, the supply of paint already delivered to the trench through the aperture is progressively depleted by deposit on the advancing strip surface, and occupies a progressively short portion of the trench (measured along the trench length); accordingly, the coating portion a, b, or c produced by deposit of paint from that aperture becomes progressively narrower along the length of the strip. At the same time, paint continuing to be delivered through one or both of the other apertures progressively occupies a greater portion of the trench length (so that the trench continues to be entirely filled with paint), and in consequence, the coating portion or portions produced by deposit of paint from such other apertures will exhibit progressive widening along the length of the strip in correspondence with the narrowing of the first-mentioned coating portion. Thus, by alternate and sequential shutoff and resumption of paint flow through the three apertures, there is achieved alternate widening and narrowing of three coating portions a, b and c along the strip length, while the overall width of the coating remains constant.

As any one of the coating.portions a, b and c becomes wider or narrower, the striations contained therein are progressively displaced transversely of the strip, so that (as indicated at 176a in Figure 17) they appear to extend diagonally rather than parallel to the long edges of the strip, although (as further indicated at 176a) typically each such diagonal striation is constituted of a staggered array of short parallel striations; as at present believed, this progressive transverse displacement of the striations in the produced coating is a result of progressive axial expansion or compression of the helical flows within the trench incident to the described selective shutoff and resumption of paint supply through the several apertures. In addition to the change in orientation of the striations, the widening or narrowing of the coating portion produces progressive variation in the spacing between adjacent striations and in the degree of blending of the two colours of paint (with consequent variation in apparent width of the striations), all in conformity with the appearance of natural wood grain. Thereby, highly effective stimulation of wood grain can be achieved in the produced pattern.

The plate 180 is provided with lateral projections 206 to facilitate mounting of the plate on appropriate support structure for holding the plate fixed in relation to the axis of the roll 172. The mounting for the plate may include means (not shown) for adjusting the spaced position of the plate relative to the roll axis, thereby to vary the gap defined between the roll surface and the plate surface 182, as may be desired to accommodate strip of different gauges and/or to change the wet thickness of the applied coating layer.

While the coating system of Figures 17 and 18 has been described as operated to produce a striped or striated coating, it is to be understood that this system is applicable as well to the production of a single-colour coating, with the advantages already noted that the coating is _{'} characterized by superior smoothness and uniformity owing to the prevention of entrapment of air (a result, inter alia, of the feature of maintaining the trench continuously entirely filled with liquid coating material under positive pressure), and that abrasion is avoided because the surface of the back-up roll moves in the same direction and at the same rate as the advancing strip. For production of a single-colour coating, only one wet coating material is delivered to the trench, and such delivery can be effected through only a single one of the paint-delivery apertures, i.e. with supply of paint through the associated main bore; indeed, in such case the apparatus can be provided with a single (e.g. centrally located) aperture and an associated single main bore, the transverse bore and the other apertures (with their associated main bores) being omitted.

In the coating line schematically shown in Figure 19, incorporating the coating device 174 of Figures 17 and 18, the aluminium strip 170 to be coated is continuously advanced (by suitable and e.g. conventional strip-advancing means) longitudinally parallel to its long dimension from a coil (not shown) around rolls 211 and a guide roll 212, and thence over the back-up roll 172 (rotatably supported, with roll 212, in a frame 215) and a further roll 216. At a locality at which the strip is held against the back-up roll, paint is applied to the outwardly facing major surface 178 of the strip from the coating device 174, to establish on the strip surface 178 a continuous layer or coating of the paint. Beyond the roll 216, the strip is passed through an oven 220 to dry the coating, and thereafter coiled again e.g. on a driven rewind roll (not shown) which, in such case, constitutes the means for advancing the strip through the coating line; within the oven, the advancing strip is in catenary suspension, and the weight of the suspended portion holds the strip against the back-up roll 172. The direction of strip advance through the coating line is indicated by arrows 221.

As will be understood from the foregoing description of Figures 17 and 18, the coating device 174 includes the plate 180 having a reservoir trench (not shown in Figure 19) with an open long side which extends, transversely of the path of strip advance, from end to end of the trench. The back-up roll 172 supports the strip surface 178 in proximate facing relation to the open side of the trench as the strip passes the trench.

As shown in Figure 19, the plate 180 is preferably so disposed that it trench, facing back-up roll 172, lies substantially in a horizontal plane containing the axis of rotation of the back-up roll, and the coating line is so arranged that the strip is held against the back-up roll at this locality, which is thus the locality at which paint is applied to the strip. It sill be understood that in continuous coating of strip, successive lengths of strip are usually joined together (spliced) endwise at a transverse seam which is thicker than the strip gauge; when this seam passes between the plate - 180 and roll 172, the plate must be temporarily moved away from the roll sufficiently to accommodate the thickness of the seam. If, for example, the plate 180 were located above the roll 172, so that the trench opened downwardly, such movement of the plate away from the roll would cause the paint then contained in the trench to be dumped on the passing strip surface, resulting in unsatisfactory coating of the strip for many feet beyond the seam. The disposition of the plate shown in Figure 19 largely obviates this problem because paint in the trench, when released by movement of the plate away from the strip, falls into a drip pan 180a rather than onto the strip surface, and therefore does not interfere with resumed application of a satisfactory coating layer upon return of the plate to operative position. In consequence, production of unacceptably coated scrap strip is advantageously minimized.

Although the plate structures described above define trenches having fixed ends, and thus a fixed length, it is advantageous to enable the length of the trench to be adjusted, thereby to vary the width of the applied coating e.g. to facilitate use of the same apparatus to coat strips of different widths. Figure 20 illustrates schematically a plate 222 having a surface 224 in which is formed an elongate, axially rectilinear trench 226 supplied with paint through an aperture 228, for use in the same manner as the plates described above in applying a coating to a strip article. The trench 226 extends for the full length of the plate, opening through the opposite sides thereof, and is closed at its ends by a pair of shutter members 230 which are snugly but slidably inserted into the opposed extremities of the trench. Means (e.g. clamps, not shown, secured to the plate 222 and adjustably engaging the shutter members) may be provided for holding the shutter members in any desired position. The length of the trench, and consequently the width of the applied coating, can be varied as desired by moving the shutter members longitudinally toward or away from each other within the trench. Thus, for example, in the coating of metal strip for use in making sliding panels, the coating layer width can readily be selected to be somewhat less than the strip width, so that both longitudinal edge portions of the coated strip surfaces are left bare to permit direct metal-to-metal contact between adjacent courses of panels (i.e. when the panels are formed, cut, and installed on a building wall) as is desired to render the panel assembly electrically conductive.

In addition to providing the beneficial results already discussed, the above-described coating systems and procedures (especially those embodiments wherein the paint or other liquid coating material is supplied under pressure to a fully enclosed reservoir or trench which is maintained entirely filled withe the liquid) afford other important advantages, with respect to operating economy and efficiency and environmental considerations, as compared to conventional roll-coating systems. The mechanical simplicity of the present systems, which have no coating rolls to maintain, reduces capital investment and maintenance costs as well as saving the energy required to rotate coating rolls. Since the systems are fully enclosed, i.e. applying a coating directly from an enclosed trench to which the paint is supplied under pressure, there is no exposed or visible paint (in open reservoirs or on rolls); hence contamination with dirt is minimized, and splashing or dripping of paint is avoided, so that the operation is advantageously clean and waste of paint is minimized. For the same reason, coatings having a high solids content (and a correspondingly low solvent content) can be applied at high line speeds, whereas with conventional rollers centrifugal effects restrict the speeds at which high solids coatings can be applied. Such rapid application of high-solids coatings and reduced use of solvent is both economically and environmentally beneficiat: Coating colour changes can be effected much more rapidly, and with production of much less scrap (strip that passes the coating station and is not satisfactorily coated during a colour change), than in the case of roll coating operations, which require relatively lengthy cleanup and reset times for colour changes. Thus, the present systems facilitate production of special colour coatings in short runs.

Moreover, the present systems achieve smoother, finer-textured coatings than are produced by roll-coating, owing in particular (as at present believed) to the extended surface or land which the coated strip passes immediately beyond the trench. Problems of blistering due to air entrapment, a cause of much poor or unsatisfactory coating in conventional operations, are eliminated by the long land and by the application of the coating material under pressure in a fully filled and enclosed trench. A still further advantage is that (as already mentioned) the width of the applied coating can be made narrower than the strip; and there is no build-up of a relatively thick bean of coating material along the edges of the coated strip, as occurs in conventional roll coating. Since the bead, if present, interferes with proper recoiling of the coated strip unless special measures (e.g. involving periodic axial movement of the recoil drum) are taken to accommodate it, the avoidance of bead formation is especially desirable.

Figures 21 to 33 show modified forms of the apparatus illustrated in Figures 1 to 3, and components corresponding to those in Figures 1 to 3 are indicated by the same reference numerals.

In the embodiment of Figures 21 to 23, a plurality of small apertures 36 (five being shown) are provided in the upper plate 18, opening downwardly through the wall 26 into the gap defined between that wall and the coated strip surface 10, beyond the dam 32, at locations spaced across the width of the surface 10. These apertures all communicate with a manifold trough 338, illustrated as formed in the plate 18 and closed by a. cover 340. In the practice of the present process, the trough 338 is maintained entirely filled with a second liquid coating material (e.g. differing in colour from the aforementioned first liquid coating material (supplied under pressure from a source represented as a pump 342, although again, the second liquid coating material could be supplied by gravity feed under hydrostatic pressure.

Specifically, the second liquid coating material is delivered to the gap between the wall 26 and the strip surface 10 (i.e. at five spaced locations, via the apertures 336) under pressure sufficient to locally. displace the first liquid coating material of the wet coating layer which already fills the gap, thereby to establish in the coating layer a longitudinal stripe 344 at the location of each of the apertures. This displacement occurs because of the selected supply pressure of the second liquid coating material and because the already-applied layer of the first liquid coating is still wet, having been maintained fully enclosed by the plate assembly at and downstream of the dam 32. It is believed that the effect of this displacement acts in an upstream direction, i.e. toward the reservoir trench 22, rather than laterally, as there is substantially no observed lateral displacement or leakage of coating material; in any event, owing to the displacement of the first liquid coating material by the second at the locations of the apertures 336, the resultant stripes 344 extend substantially entirely through the thickness of the produced coating rather than merely overlying the layer of the first coating material. Consequently, the stripes do not wear preferentially or disappear prematurely upon weathering.

The stripes 344 of the second liquid coating material re narrow and sharply defined, extending parallel to each other from the five apertures 336, and exhibit very little if any blending with the first liquid coating material. Some degree of blending along the stripes may be effected, if desired, by providing a movable portion of the wall 26 downstream of the apertures 336 and moving that wall portion, in the plane of the wall, transversely of the direction of strip advance. To this end, in the apparatus of Figures 21 to 23, the upper plate 18 has a circular recess 346 opening downwardly through the surface of wall 26 downstream of the apertures 336; within this recess is disposed a disc 348, very slightly smaller than the recess in diameter, having a downwardly facing surface coplanar with and effectively constituting a part of the wall 26. The disc is mounted (by means of a shaft 3350 projecting upwardly through a bore in the plate 18) for angular displacement about an axis perpendicular to the plane of wall 26. The diameter and location of the disc are such that the disc surface is traversed by, and thus in contact with, the five stripes 344 emerging from the apertures 336. Angular dis- . placement of the disc about the aforementioned axis moves its downwardly facing surface in the plane of the wall 26 with a component of motion transverse to the direction of strip advance; the resultant drag on the disc-engaging surface of the wet coating layer causes some blending of the two coating materials along the stripes, as may be desired for particular pattern effects.

The embodiment of Figures 24 to 28 differs from that of Figures 21 to 23 in that the apertures for delivering the second liquid coating material to the gap between the strip being coated and the facing wall are angularly displaceable about an axis perpendicular to the plane of the coated strip surface 10. Thus, a disc 352 is disposed in a circular recess 354 which is formed in the upper plate 18 and which opens downwardly through the wall 26 downstream of the trench 22 in the path of strip advance, the disc being only slightly smaller in diameter than the recess. The disc 352, mounted (by means of a shaft 356 that projects upwardly through a bore in plate 18) for rotation about an axis perpendicular to wall 26, has a lower surface 358 coplanar with and effectively constituting part of the wall 26. Five coating material delivery apertures 336, formed in the disc 352, open through the surface 358 into the gap, and communicate with an enclosed manifold passage or trough 238a also formed within the disc 352. In this embodiment, the second liquid coating material is supplied under pressure to the trough 338a through a passage 360 in the disc shaft 358.

When the disc 352 is stationary, and oriented as shown in Figure 24, with the apertures 336a aligned in a horizontal line perpendicular to the direction of strip advance, performance of the present process proceeds as described above with reference to Figures 1 to 3, and the five apertures produce five parallel longitudinal stripes of the second liquid coating material in a coating layer otherwise constituted of the first liquid coating material delivered to trench 22, it being understood that the second coating material is delivered through the apertures 336a under pressure sufficiently to locally displace the first liquid coating material in the wet coating layer. If, however, during continuous advance of the strip 11, and continuous supply of the two liquid coating materials to the apparatus, the disc 352 is rotated about the axis of shaft 356, the apertures 336a (though fixed in position relative to each other) are angularly displaced about that axis, with resultant change in location and spacing of the produced stripes. Thus, for example, rotation of the disc 352 through 45° from the position shown at A in Figure 28 to the position shown at B in Figure 28 causes the stripes 44 to change progressively, in location and spacing, from the initial condition shown at 344a in Figure 28 to the final condition shown at 344b in Figure 28, in correspondence with the angular change in position of the apertures relative to the path of strip advance. In this way, diversified pattern effects, with wandering, diverging, and converging stripes can be achieved.

As indicated in Figures 26 and 27, each aperture 336a may have an associated short groove 362, tapering in depth and width away from the aperture, and formed in the lower surface 358 of the disc 352 so as to be in contact with the wet coating layer. These grooves, positioned to extend usually or generally in a downstream direction from their respective associated apertures, serve to impart a fine flecked appearance or texture to the coating in and adjacent the produced stripes.

There is no separate blending disc 348 in the apparatus of Figures 24 to 28, but the movement of the surface 358 of disc 352, in those portions which engage the wet coating layer downstream of the apertures 336a, has a like blending effect. In addition, at those portions of the coating layer where one or more stripes are oriented diagonally to the direction of strip advance owing to progressive movement of the disc 352, drag of the fixed portion of wall 26 (downstream of the disc) on the wet coating layer produces some blending along the stripes.

Figures 29 to 33 illustrate a specific embodiment of the invention (currently preferred for production of a coating with a simulated wood grain pattern) of the general type shown in Figures 24 to 28, i.e. having plural coating material delivery apertures carried in a rotatably mounted disc. The apparatus includes a top plate 18 and a bottom plate 20 secured together at their corners by bolts 421a, with biasing springs 421b provided for maintaining the plates in spaced-apart relation and lateral guides or stops 421c projecting upwardly from the lower plate to assure proper register of the plates.

A plurality of coating material delivery apertures 436 with associated manifold passages 438 are formed in a disc 452 which is received in a downwardly opening circular recess 454 in the plate 18. This disc has an upwardly projecting vertical shaft 456 and a smooth downwardly facing plane surface 458 that is disposed in coplanar relation to the plate surface 26, downstream of the dam 32, to constitute a portion of the wall facing the coated major surface of a strip article advancing in the direction indicated by arrows 431 through the gap 30. The apertures 436 open downwardly through the disc surface 458 for delivery, to the coating-filled gap between the wall and the coated strip surface, of a second liquid coating material which is delivered under pressure from a suitable source (not shown) through a passage 460 in the shaft 456 to the manifold passages 438.

The shaft 456 is journalled in a bearing structure 462, mounted atop the plate 418, to support the disc 452 for rotation about an axis perpendicular to the plane of the wall constituted by surfaces 26 and 458. It will be understood that the disc 452, with its apertures 436 and manifold passages 438, corresponds generally in structure and function to the disc 352 of the embodiment of Figures 24 to 28, providing delivery of second liquid coating material to the aforementioned gap under pressure through plural spaced apertures while being rotatable to effect angular displacement of the apertures for varying the positions and spacing of the stripes produced by such delivery of the second coating material. As best seen in Figures 31 to 33, the disc 452 can be a circular metal plate through which the manifold passages 438 are bored; the aperture 436 are drilled into the passages 438 through the lower surface of the plate, and the ends of the passages 438 are then closed by suitable means as indicated at 464.

From Figure 31, it will be seen that the apertures 436 are distributed across one half of the downwardly facing surface of the disc 452 and are aligned in four rows each comprising four spaced apertures. The rows are arranged at angles to each other in the form of the letter W and are all eccentric with respect to the disc; i.e. a line interconnecting any row of four apertures does not pass through the centre of the disc. This arrangement of apertures is found particularly effective for producing a simulated wood-grain pattern of stripes of the second coating material delivered thereto, when the disc is progressively angularly displaced first in one direction and then in the opposite direction during the course of a coating operation; that is to say, with this arrangement of apertures, there are produced a series of narrow stripes individually resembling the lines of a wood-grain pattern and varying progressively in position and spacing, with angular displacement of the disc, in a manner corresponding to that of natural wood-grain lines. The manifold pattern associated with the various rows all interconnect with each other and, by further passages 438a (also bored through the disc and sealed at their outer ends), are interconnected with the passage 460.

As will be understood, in use of the apparatus of Figures 29 to 33 to coat a strip article with a coating having a simulated wood-grain pattern, the article is continuously advanced along the path indicated by arrows 131 through the gap 30 while a first liquid coating material is delivered under pressure to the trough 22 so as to maintain the trough entirely filled therewith, and while a second liquid coating material is delivered to the manifold passages of the disc 452 under pressure and thence through the apertures 436, with progressive angular displacement of the disc, first in one direction and then in another. The movement of the disc causes the disc surface, in contact with the coating layer, to effect some degree of blending or mixing of the two liquid coating materials downstream of the apertures 436 to enhance further the resemblance to wood-grain lines.

For satisfactory coating operation, it is critical that the disc surface 458 be located very precisely in the plane of the plate surface 26. To facilitate proper mounting of the disc, and this requisite positioning of the surface 458, a series of stops 470 are disposed within the recess 454 and threaded in the plate 18 so as to be vertically adjustable. The stops bear against the upper surface of the disc 452 for establishing the vertical position of the disc relative to surface 26.

One particularly convenient arrangement for achieving proper adjustment of the disc position, shown in Figures 29 and 30, includes an array of permanent magnets 472 mounted in the plate 18 so as to project into the recess 454 above the disc and to attract the disc (which, in this arrangement, is fabricated of a magnetic metal) upwardly into engagement with the stops 470. Although the magnets 472 do not actually engage the disc, their attraction holds it against the stops, which may then readily be adjusted to assure the requisite coplanar arrangement of the surfaces 458 and 26.

## Claims

1. Apfocess for coating a major surface (10) of a strip article (11) of indeterminate length, including the steps of continuously advancing the article longitudinally past a dam (32) extending transversely of said major surface in adjacent spaced relation thereto while supplying a flowable liquid coating material to said major surface immediately ahead of said dam and, immediately beyond said dam, advancing said article longitudinally past a wall (26) of extended length in the direction of strip advance (46) and facing said major surface, said strip being uniformly restrained by restraining means (20; 122) against movement of said major surface away from said wall (26) beyond a predetermined distance equal to a desired wet thickness of said coating material on said major surface characterised in that the said wall of extended length is provided by a rigid member (18; 120) which wall is equidistantly spaced from a rigid support constituting the restraining means (20; 122), said rigid member being fixedly securable relative to the restraining means.

2. A process according to claim 1, characterised in that said article (11) is restrained as aforesaid by a second wall (20) spaced uniformly from the first-mentioned wall (26) of extended length to define therewith a gap (30) through which the article (11) passes, and in that said article (11) passing through said gap (30) moves relative to both of said walls (26, 20).

3. A process according to claim 1 or claim 2, characterised in that the step of supplying the coating material includes supplying coating material of differing compositions to different portions of said major surface across the width thereof ahead of said dam (32).

4. A process according to claim 3, characterised in that said different compositions of coating material differ from each other in colour.

5. A process according to claim 3 or claim 4, characterised by the step of varying the supply of different coating material compositions to said major surface immediately ahead of said dam for producing variations in coating appearance along the length of said major surface.

6. A process according to any one of claims 1 to 6, characterised in that further wet flowable coating material is supplied to said major surface at one or more locations (112) downstream of the dam, which further coating material is of different composition to that applied upstream of the dam.

7. A process as claimed in claim 1, characterised in that said article is restrained as aforesaid by an endless surface (122) moving continuously in the same direction and at the same rate as said article.

8. A process according to claim 7, characterised in that a fully enclosed reservoir (184) of said coating material is provided immediately ahead of said dam and said coating material is delivered to said reservoir (184) under positive pressure for maintaining said reservoir entirely filled therewith.

9. A process according to claim 1, further characterised by the step of delivering, through at least one aperture (336) in said wall of extended ' length, at least one further liquid coating material to said gap under pressure sufficient to displace locally the first said liquid coating material in the wet coating layer which is already on said major surface, thereby to establish a stripe (344) of the second liquid coating material in the coating layer (12).

10. A process according to claim 9, characterised in that said first and further coating materials are pigmented, and differ from each other in pigmentation, such that said stripe is visibly distinguishable from portions of said coating layer constituted of said first coating material.

11. A process according to claim 9 or claim 10, further characterised by the step of selectively moving a portion of said wall of extended length, beyond said one aperture, in a direction parallel to said major surface and transverse to the direction of article advance, during advance of the article and delivery of said further coating material through said one aperture, for effecting blending of said first and further coating materials in and adjacent said stripe.

12. A process according to claim 11, characterised in that said wall (26) of extended length is planar and has a movable portion comprising a disk (348) rotatable about an axis perpendicular to the plane ofthewall, and wherein the moving step comprises effecting annular movement of said disk about said axis.

13. A process according to claim 9, further characterised by the step of moving said one aperture (336a) in a direction parallel to said major surface and transverse to the direction of article advance, during advance of the article and delivery of said further coating material through said one aperture, for progressively changing the location of said stripe (344b), along the length of said article, relative to the sides of said article.

14. A process according to claim 13, characterised in that said wall (26) of extended length is planar and has a movable portion comprising a disc (352) rotatable about an axis perpendicular to the plane of the wall, said one aperture being located in said disc, and in that the moving step comprises effecting angular movement of said disc about said axis.

15. A process according to claim 9, characterised in that said further liquid coating material is delivered to said gap under pressure as aforesaid through a plurality of apertures (336a) spaced apart in said wall transversely of the direction of strip advance, thereby to establish a corresponding plurality of stripes of said further liquid coating material in said coating layer.

16. A process according to claim 15, further characterised by the step of progressively moving said apertures, parallel to said major surface and transversely of the direction of article advance, during advance of the article and delivery of said further coating material, for progressively varying the locations of the stripes, along the length of the article relative to the sides of the article.

17. A process according to claim 16, characterised in thatthe aperture-moving step comprises moving the apertures for progressively varying the spacing between the stripes.

18. A process according to claim 17, characterised in that said wall (26) of extended length is planar and has a movable portion comprising a disc rotatable about an axis perpendicular to said major surface, said apertures being located in said disc, and the aperture-moving step comprises angularly displacing said disc about said axis.

19. A process according to claim 18, characterised in that said apertures are aligned in a plurality of rows (438) eccentric to said axis, with at least one of said rows oriented at an acute angle with respect to at least one other of said rows.

20. Apparatus for forming a continuous adherent coating layer (12) on a major surface (10) of a strip article (Tl7 of indeterminate length comprising means defining a path of advance (46) of said article lengthwise of itself including an extended wall (26) facing said major surface of said article and so arranged that the advancing article moves longitudinally relative thereto and means (20; 122) for uniformly restraining said article against movement of said major surface (10) away from said wall beyond a predetermined distance during advance of said article past said wall, means constituting a dam (32) extending transversely of the path of article advance so as to be disposed in adjacent spaced relation to said major surface of the article and means (22) for supplying a wet flowable coating material to said major surface ahead of said dam, characterised in that said extended wall (26) is constituted by a surface of a rigid member (18; 120) which surface is equidistantly spaced from a rigid support constituting the said restraining means and in that means (42) are provided for fixedly securing said rigid member (18; 120) relative to said restraining means.

21. Apparatus as claimed in claim 20, characterised in that the end of said extended wall remote from said one end is formed as a sharp edge (47) for preventing cavitation of wet coating material on said major surface advancing beyond the wall.

22. Apparatus as claimed in claim 20 or 21, characterised in that the dam (32) at said one end of said wall has a surface gradually and progressively approaching said wall in the direction of strip advance.

23. Apparatus as claimed in any one of claims 20 to 22 characterised in that said members are in the form of plates (18, 20) and in that a surface portion of one of said plates at the inlet end of the space between the plates constitutes said dam.

24. Apparatus as claimed in claim 23 characterised in that said securing means (42) is adjustable for varying the spacing between said facing surfaces of said plates.

25. Apparatus as claimed in any one of claims 20 to 24, characterised in that the coating material supplying means includes means for delivering at least two different coating material compositions to different portions of said major surface ahead of said dam.

26. Apparatus as claimed in any one of claims 20 to 22 characterised in that said restraining means comprises an endless surface movable in the same direction and at the same rate .as a strip article advancing in said path.

27. Apparatus as defined in claim 26, characterised in that said restraining means comprises a rotatably mounted roll (122) having a cylindrical periphery constituting said endless surface and in that said wall (128) is curved in conformity with the roll periphery.

28. Apparatus as claimed in claim 27, characterised in that said roll (122) is mounted for rotation about an axis parallel to and lying generally in the same common horizontal plane as the dam (136), and in that said wall (128) is movable horizontally toward and away from said roll (122).

29. Apparatus as claimed in any one of claims 20 to 28, characterised in that said supplying means comprises means for establishing and maintaining an enclosed reservoir of wet flowable coating material ahead of an in contact with said dam.

30. Apparatus as claimed in claim 29, further characterised by means (230) for varying the length of said reservoir in a direction transversely of the strip.

31. Apparatus as claimed in claim 29 or claim 30, characterised in that said reservoir is in the form of an elongate trench (184) opening toward said article major surface along the length of said dam and otherwise fully enclosed, and in that means (202a) is provided for supplying said coating material under positive pressure to said trench (184) to maintain said trench entirely filled therewith.

32. Apparatus as claimed in any one of claims 20 to 24 further characterised by means for delivering, through at least one aperture in said wall, to at least one locality in said gap, a further liquid coating material under pressure sufficient to displace locally the first liquid coating material in the coating layer, thereby to establish a stripe (344) of said further liquid coating material in the coating layer (12).

33. Apparatus as claimed in claim 32, characterised in that said extended wall is planar and includes a portion constituted by a disc (452) having a surface copolanar with said wall and in that a plurality of said apertures open through said disc surface at spaced locations, said disc being mounted for rotation about an axis perpendicular to said wall, means being provided for supplying said further liquid coating material under pressure through said apertures.

34. Apparatus as claimed in claim 33, characterised in that said apertures (436) are aligned in at least one row eccentric to said axis.

35. Apparatus as claimed in claim 33 or claim 34, characterised in that structure having an extended planar surface constituting a fixed portion of said extended wall (26), and with a transverse edge constituting said dam, has a circular recess (454) within which said disc is received, said disc being fabricated of magnetic material and in that there is provided stop means (470) projects into said recess to bear against said disc and is adjustably mounted in said structure for movement in a direction perpendicular to the plane of said extended wall (26) to position said disc surface in coplanar relation to said fixed wall portion; and magnet means (472) mounted in said structure for attracting said disc into engagement with said stop means.

36. Apparatus as claimed in claim 32, characterised in that said wall has a groove (362) formed therein, extending from said one aperture generally in the direction of advance of said article.

## Patentansprüche

1. Verfahren zum Beschichten einer Hauptfläche (10) eines streifenförmigen Gegenstandes (11) von unbestimmter Länge, welches folgende Schritte enthält: kontinuierliches Vorschieben des Gegenstandes in Längsrichtung vorbei an einem Damm (32), welcher sich quer zur genannten Hauptfläche, dieser mit Abstand benachbart erstreckt, während ein fließfähiges flüssiges Beschichtungsmaterial der genannten Hauptfläche unmittelbar vor dem genannten Damm und unmittelbar über den genannten Damm hinaus zugeführt wird, Vorschieben des genannten Gegenstandes in Längsrichtung vorbei an einer Wand (26) von in Richtung des Streifenvorschubes (46) ansgedehnter Länge, welche Wand der genannten Hauptfläche zugewendet ist, wobei der Streifen von Festhalteeinrichtungen (20; 122) gegen Bewegungen der genannten Hauptfläche von der genannten Wand (26) weg über einen bestimmten Abstand hinaus, welcher einer gewünschten nassen Dicke des genannten Beschichtungsmaterial auf der -genannten Hauptfläche gleich ist, gleichförmig festgehalten ist, dadurch gekennzeichnet, daß die genannte Wand von ausgedehnter Länge von einem starren Glied (18; 120) gebildet ist, welche Wand äquidistant von einer starren Unterstützung entfernt ist, welche die Festhalteeinrichtung (20; 122) bildet, wobei das genannte starre Glied relativ zu den Festhalteeinrichtungen unverrückbar befestigbar ist.

2. Verfahren nach Anspruch 1, dadurch gekennzeichnet, daß der genannte Gegenstand (11) wie vorhin erwähnt von einer zweiten Wand (20) festgehalten ist, welche gleichförmig von der erstgenannten Wand (26) von ausgedehnter Länge entfernt ist, um mit dieser einen Spalt (30), durch welchen der Gegenstand (11) hindurchläuft, zu bilden, und dadurch, daß der genannte Gegenstand (11), welcher durch den genannten Spalt (30) hindurch läuft, sich relativ zu den beiden genannten Wänden (26, 20) bewegt.

3. Verfahren nach Anspruch 1 oder Anspruch 2, dadurch gekennzeichnet, daß der Schritt des Zuführens des Beschichtungsmaterials das Zuführen von Beschichtungsmaterialien verschiedener Zusammensetzung zu verschiedenen Abschnitten der genannten Hauptfläche quer über deren Breite vor dem genannten Damm (32) enthält.

4. Verfahren nach Anspruch 3, dadurch gekennzeichnet, daß die verschiedenen Zusammensetzungen von Beschichtungsmaterialien sich voneinander in der Farbe unterscheiden.

5. Verfahren nach Anspruch 3 oder Anspruch 4, gekennzeichnet durch den Schritt die Zuführung von verschiedenen Beschichtungsmaterialzusammensetzungen zu der genannten Hauptfläche unmittelbar vor dem genannten Damm zu variieren, um Veränderungen im Aussehen der Beschichtung entlang der ganzen Länge der genannten Hauptfläche zu erzeugen.

6. Verfahren nach einem der Ansprüche 1 bis 5, dadurch gekennzeichnet, daß nasses fließfähiges Beschichtungsmaterial der genannten Hauptfläche an einer oder mehreren Stellen (112) stromabwärts von Damm zugeführt wird, welches weitere Beschichtungsmaterial von unterschiedlicher Zusammensetzung gegenüber jenem stromaufwärts vom Damm aufgebrachten Beschichtungsmaterial ist.

7. Verfahren nach Anspruch 1, dadurch gekennzeichnet, daß der Gegenstand wie vorhin erwähnt von einer endlosen Oberfläche (122) festgehalten ist, welche sich kontinuierlich in der gleichen Richtung und mit der gleichen Geschwindigkeit wie der genannte Gegenstand bewegt.

8. Verfahren nach Anspruch 7, dadurch gekennzeichnet, daß ein gänzlich geschlossenes Reservoir (184) des genannten Beschichtungsmaterials unmittelbar vor dem genannten Damm vorgesehen ist und daß das genannte Beschichtungsmaterial dem genannten Reservoir (184) unter Überdruck zugeführt wird, um das genannte Reservoir gänzlich damit gefüllt zu halten.

9. Verfahren nach Anspruch 1, weiters gekennzeichnet durch den Schritt, zumindest durch eine Öffnung (336) in der genannten Wand von ausgedehnter Länge zumindest ein weiteres flüssiges Beschichtungsmaterial dem genannten Spalt unter einem Druck zuzuführen, der ausreicht das erstgenannte flüssige Beschichtungsmaterial in der nassen Beschichtungsschichte, welche sich bereits auf der genannten Hauptfläche befindet, lokal zu verdrängen, wodurch ein Streifen (344) des zweiten flussigen Beschichtungsmaterials auf der Beschichtungschicht (12) gebildet wird.

10. Verfahren nach Anspruch 9, dadurch gekennzeichnet, daß das genannte erste und die weiteren Beschichtungsmaterialien pigmentiert sind und sich voneinander in der Pigmentation unterscheiden, sodaß der genannte Streifen von Abschnitten der genannten Beschichtungsschicht, welche von dem genannten ersten Beschichtungsmaterial gebildet ist, sichtbar unterscheidbar ist.

11. Verfahren nach Anspruch 9 oder Anspruch 10, weiters gekennzeichnet durch den Schritt, einen Teil der genannten Wand von ausgedehnter Länge außerhalb der genannten einen Öffnung in einer zu der genannten Hauptfläche parallelen Richtung und quer zur Richtung des Gegenstandsvorschubes zu bewegen, während des Vorschubes des Gegenstandes und der Abgabe des genannten weiteren Beschichtungsmaterials durch die genannte eine Öffnung, um eine Vermischung des genannten ersten und weiteren Beschichtungsmaterials in und neben dem genannten Streifen zu erreichen.

12. Verfahren nach Anspruch 11, dadurch gekennzeichnet, daß die Wand (26) von ausgedehnter Länge eben ist und einen bewegbaren Teil mit einer Scheibe (348), welche um eine zur Ebene der Wand senkrechte Achse drehbar ist, enthält, wobei der Bewegungsschritt das Bewirken einer ringförmigen Bewegung der genannte Scheibe um die genannten Achse enthält.

13. Verfahren nach Anspruch 9, weiters gekennzeichnet durch den Schritt, die genannte eine Öffnung (336a) in einer Richtung parallel zu der genannten Hauptfläche und quer zur Richtung des Gegenstandsvorschubes während des Vorschubes des Gegenstandes und der Abgabe des genannten weiteren Beschichtungsmaterials durch die genannte eine Öffnung zu bewegen, um den Ort des genannten Streifens (344b) entlang der Länge des genannten Gegenstandes relativ zu den Seiten des genannten Gegenstandes fortschreitend zu verändern.

14. Verfahren nach Anspruch 13, dadurch gekennzeichnet, daß die genannte Wand (26) von ausgedehnter Länge eben ist und einen bewegbaren Teil aufweist, welcher eine Scheibe (352), die um eine zur Ebene der Wand senkrechte Achse drehbar ist, enthält, wobei die genannte eine Öffnung in jener Scheibe angebracht ist und dadurch gekennzeichnet, daß der Bewegungsschritt das Bewirken einer Winkelbewegung der genannten Scheibe um die genannte Achse enthält.

15. Verfahren nach Anspruch 9, dadurch gekennzeichnet, daß das weitere flüssige Beschichtungsmaterial dem genannten Spalt wie vorhin erwähnt unter Druck durch eine Mehrzahl von Öffnungen (336a) zugeführt wird, welche Öffnungen in der genannten Wand quer zur Richtung des Streifenvorschubes mit Abstand voneinander angebracht sind, wodurch eine entsprechende Mehrzahl von Streifen des genannten weiteren flüssigen Beschichtungsmaterials in der genannten Beschichtungsschicht erzeugt wird.

16. Verfahren nach Anspruch 15, ferner gekennzeichnet durch den Schritt, die genannten Öffnungen progressiv parallel zu der genannten Hauptfläche und quer zur Richtung des Gegenstandsvorschubes während des Vorschubes des . Gegenstandes und der Zuführung des genannten weiteren Beschichtungsmaterials zu bewegen, um den Ort der Streifen entlang der Länge des Gegenstandes relativ zu den Seiten des Gegenstandes progressiv zu verändern.

17. Verfahren nach Anspruch 16, dadurch gekennzeichnet, daß der Öffnungsbewegungsschritt das Bewegen der Öffnungen zur progressiven Änderung des Abstandes zwischen den Streifen enthält.

18. Verfahren nach Anspruch 17, dadurch gekennzeichnet, daß die genannte Wand (26) von ausgedehnter Länge eben ist und einen bewegbaren Teil aufweist, welcher eine um eine zu der genannten Hauptfläche senkrechte Achse drehbare Scheibe enthält, wobei die Öffnungen in der genannten Scheibe angebracht sind und der Öffnungsbewegungsschritt das Verschieben der genannten Scheibe um die genannte Achse dem Winkel nach enthält.

19. Verfahren nach Anspruch 18, dadurch gekennzeichnet, daß die genannten Öffnungen in einer Mehrzahl von Reihen (438) ausgerichtet sind, die exzentrisch zu der genannten Achse liegen, wobei zumindest eine der genannten Reihen in einem spitzen Winkel relativ zumindest einer anderen der genannten Reihen orientiert ist.

20. Vorrichtung zur Bildung einer zusammenhängenden haftenden Beschichtung (12) auf einer Hauptfläche (10) eines streifenförmigen Gegenstandes (11) von unbestimmter Länge mit Einrichtungen, welche einen Vorschubweg (46) für diesen Gegenstand in seiner Längsrichtung definieren, welche Einrichtungen eine langgestreckte Wand (26), die der Hauptfläche des genannten Gegenstandes zugewendet und so angeordnet ist, daß der laufende Gegenstand sich relativ zu ihr in Längsrichtung bewegt, und Einrichtungen (20; 122) zum gleichförmigen Festhalten des Gegenstandes gegen Bewegungen der genannten Hauptfläche (10) von der Wand weg Über einen bestimmten Abstand hinaus während des Vorschubes des genannten Gegenstandes entlang der Wand, Einrichtungen, welche einen Damm (32), der sich quer zur Vorschubrichtung des Gegenstandes so erstreckt, daß er benachbart zur Hauptfläche in einem Abstand von dieser angeordnet ist, und Einrichtungen (22) zum Zuführen eine fließfähigen Beschichtungsmaterials zu der genannten Hauptfläche vor dem genannten Damm enthält, dadurch gekennzeichnet, daß die genannte langgestreckte Wand (26) von einer Oberfläche eines starren Gliedes (18; 120) gebildet ist, welche Oberfläche äquidistant von einer starren Unterstützung entfernt ist, welche die Festhalteeinrichtung bildet und daß Einrichtungen (42) zum unverrückbaren Befestigen des genannten starren Gliedes (18; 120) relativ zu den Festhalteeinrichtungen vorgesehen sind.

21. Vorrichtung nach Anspruch 20, dadurch gekennzeichnet, daß das Ende der ausgedehnten Wand, welches von dem genannten einen Ende abgewendet ist, als scharfe Kante (47) ausgebildet ist, um Kavitation des nassen Beschichtungsmaterials auf der genannten Hauptfläche, welche über die Wand hinaus vorrückt, zu verhindern.

22. Vorrichtung nach Anspruch 20 oder 21, dadurch gekennzeichnet, daß der Damm (32) an dem genannten einen Ende der genannten Wand eine Oberfläche besitzt, welche sich graduell und progressiv an die genannte Wand in Richtung des Streifenvorschubes annähert.

23. Vorrichtung nach einem der Ansprüche 20 bis 22, dadurch gekennzeichnet, daß die genannten Glieder die Form von Platten (18, 20) besitzen und daß ein Oberflächenteil einer der genannten Platten am Einlaßende des Zwischenraumes zwischen den Platten den genannten Damm bildet.

24. Vorrichtung nach Anspruch 23, dadurch gekennzeichnet, daß die Festhalteeinrichtung (42) einstellbar ist, um den Abstand zwischen den einander zugewendeten Flächen der genannten Platten zu νerändern.

25. Vorrichtung nach einem der Ansprüche 20 bis 24, dadurch gekennzeichnet, daß die Zuführeinrichtungen für das Beschichtungsmaterial Einrichtungen zur Zuführung von mindestens zwei verschiedenen Beschichtungsmaterialzusammensetzungen zu verschiedenen Teilen der genannten Hauptfläche vor dem genannten Damm enthalten.

26. Vorrichtung nach einem der Ansprüche 20 bis 22, dadurch gekennzeichnet, daß die Festhalteeinrichtungen eine endlose Oberfläche enthalten, welche in der gleichen Richtung und mit der gleichen Geschwindigkeit wie der in dem genannten Pfad vorgeschobene streifenförmige Gegenstand bewegbar ist.

27. Vorrichtung nach Anspruch 26, dadurch gekennzeichnet, daß die genannten Festhalₜeein- richtungen eine drehbar gelagerte Walze (122) mit zylindrischer Peripherie enthalten, welche die genannte endlose Oberfläche bildet, und daß die genannte Wand (128) konform mit der Peripherie der Walze gekrümmt ist.

28. Vorrichtung nach Anspruch 27, dadurch gekennzeichnet, daß die genannte Walze (122) um eine Achse drehbar ist, welche parallel zum Damm (136) und im allgemeinen in der gleichen gemeinsamen Horizontalebene wie der Damm liegt, und daß die genannte Wand (128) horizontal gegen die genannte Walze (122) hin und von dieser weg bewegbar ist.

29. Vorrichtung nach einem der Ansprüche 20 bis 28, dadurch gekennzeichnet, daß die genannten Zuführeinrichtungen Einrichtungen zum Herstellen und Aufrechterhalten eines geschlossenen Reservoirs von nassem fließfähigem Beschichtungsmaterial vor dem genannten Damm und in Berührung mit jenem enthalten.

30. Vorrichtung nach Anspruch 29, weiters gekennzeichnet durch Einrichtungen (230) zur Veränderung der Länge des genannten Reservoirs in einer Richtung quer zum Streifen.

31. Vorrichtung nach Anspruch 29 oder 30, dadurch gekennzeichnet, daß das Reservoir die Form einer langgestreckten Rinne (184) besitzt, weiche sich gegen die Hauptfläche des ge--nannten Gegenstandes entlang der Länge des genannten Dammes öffnet und änderseits vollkommen geschlossen ist, und .daß Einrichtungen (202a) vorgesehen sind zur Zuführung des genannten Beschichtungsmaterials unter Überdruck zu der genannten Rinne (184), um die genannte Rinne mit diesem gänzlich gefüllt zu erhalten.

32. Vorrichtung nach einem der Ansprüche 20 bis 24, ferner gekennzeichnet durch Einrichtungen zur Zuführung eines weiteren flüssigen Beschichtungsmaterials durch mindestens eine Öffnung in der genannten Wand zumindestens einer Stelle in dem genannten Spalt unter einem Druck, welcher ausreichend ist, das zuerst genannte flüssige Beschichtungsmaterial in der Beschichtungsschicht lokal zu verdrängen, wodurch ein Streifen (344) des genannten weiteren Beschichtungsmaterials in der Beschichtungsschicht (12) gebildet wird.

33. Vorrichtung nach Anspruch 32, dadurch gekennzeichnet, daß die langgestreckte Wand eben ist und einen Teil enthält, welcher von einer Scheibe (452) mit einer Oberfläche, die koplanar mit der genannten Wand ist, enthält, und daß eine Mehrzahl der genannten Öffnungen sich durch die genannte Scheibenfläche an in Abstand stehenden Stellen öffnet, wobei die genannte Scheibe um eine zu der Wand senkrecht stehende Achse drehbar befestigt ist, und Einrichtungen vorgesehen sind für die Zufuhr des genannten weiteren flüssigen Beschichtungsmaterials unter Druck durch die genannten Öffnungen.

34. Vorrichtung nach Anspruch 33, dadurch gekennzeichnet, daß die genannten Öffnungen (436) in mindestens einer zu der genannten Achse exzentrischen Reihe ausgerichtet sind.

35. Vorrichtung nach Anspruch 33 oder 34, dadurch gekennzeichnet, daß ein Aufbau mit einer langgestreckten ebenen Oberfläche, der einen feststehenden Teil der genannten langgestreckten Wand (26) und mit einer querverlaufenden Kante den genannten Damm bildet, eine kreisförmige Vertiefung (454), innerhalb welcher die genannte Scheibe liegt, aufweist, wobei die genannte Scheibe aus magnetischem Material hergestellt ist, daß Anschläge (470) vorgesehen sind, welche in die Ausnehmung vorspringen um sich an die genannte Scheibe anzulegen und in dem Aufbau senkrecht zur Ebene der langgestreckten Wand einstellbar montiert sind, um die genannte Scheibenfläche (26) komplanar mit dem genannten feststehenden Wandteil auszurichten, und daß Magneteinrichtungen (472) in dem genannten Aufbau vorgesehen sind, um die genannte Scheibe in Anlage an die genannten Anschläge zu ziehen.

36. Vorrichtung nach Anspruch 32, dadurch gekennzeichnet, daß in der genannten Wand eine Nut (362) geformt ist, welche sich von der genannten einen Öffnung im allgemeinen in Vorschubrichtung des genannten Gegenstandes erstreckt.

## Revendications

1. Procédé pour revêtir une surface principale (10) d'un feuillard (11) de longueur indéterminée, comportant les stades d'avancement continuel du feuillard dans le sens longitudinal au-delà d'un barrage (32) s'étendant transversalement par rapport à ladite surface principale en rapport adjacent mais espacé avec celle-ci, tout en fournissant une matière de revêtement liquide coulable à ladite surface principale immédiatement devant ledit barrage et immédiatement au-delà dudit barrage, d'avancement dudit feuillard longitudinalement en regard d'une paroi (26) de longueur étendue dans le sens de l'avancement (46) du feuillard et en regard de ladite surface principale, ledit feuillard étant empêché de façon uniforme par des moyens d'empêchement (20; 122) à l'encontre d'un mouvement de ladite surface principale à l'écart de ladite paroi (26) au-delà d'une distance prédéterminée égale à l'épaisseur désirée à l'étant humide de ladite matière de revêtement sur ladite surface principale, caractérisé en ce que ladite paroi de longueur étendue est constituée par un organe rigide (18; 120), paroi qui est espacée de façon équidistante d'un support rigide constituant les moyens d'empêchement (20; 122), ledit organe rigide étant susceptible d'une fixation à demeure par rapport auxdits moyens d'empêchement.

2. Procédé selon la revendication 1, caractérisé en ce que ledit feuillard (11) est empêche, comme indiqué plus haut, par une seconde paroi (20) espacée de façon uniforme de la paroi de longueur étendue mentionnée en premier lieu (26) pour définir avec elle un intervalle (30) à travers lequel passe le feuillard (11) et en ce que ledit feuillard (11) passant par ledit intervalle (30) se déplacé par rapport aux deux parois (26, 20).

3. Procédé selon la revendication 1 ou 2, caractérisé en ce que le stade fourniture de la matière de revêtement comprend la fourniture des matières de revêtement ayant des compositions différentes à des parties différentes de ladite surface principale dans le sens de sa largeur devant ledit barrage (32).

4. Procédé selon la revendication 3, caractérisé en ce que lesdites compositions différentes de la matière de revêtement diffèrent les unes des autres par la couleur.

5. Procédé selon la revendication 3 ou 4, caractérisé en ce qu'il comporte un stade de variation de la fourniture des compositions différentes de matière de revêtement à ladite surface principale immédiatement devant ledit barrage pour obtenir des variations de l'aspect du revêtement dans le sens de la longueur de ladite surface principale.

6. Procédé selon l'une quelconque des revendications 1 à 5, caractérisé en ce qu'on fournit un supplément de matière de revêtement coulable à l'état humide à ladite surface principale en un ou plusieurs emplacements (112) en aval du barrage, ladite matière supplémentaire de revêtement étant d'une composition différente de celle appliquée en amont du barrage.

7. Procédé selon.la revendication 1, caractérisé en ce qu'on empêche, comme indiqué plus haut, ledit feuillard par une surface sans fin (122) se déplaçant continuellement dans la même direction et à la même vitesse que ledit feuillard.

8. Procédé selon la revendication 7, caractérisé en ce qu'un réservoir entièrement fermé (184) de ladite matière de revêtement est monté immédiatement devant ledit barrage et ladite matière de revêtement est débitée audit réservoir (184) sous une pression positive pour maintenir ledit réservoir entièrement rempli avec elle.

9. Procédé selon la revendication 1, également caractérisé par le stade consistant à débiter, à travers au moins une ouverture (336) dans ladite paroi de longueur étendue, au moins une autre matière de revêtement liquide audit intervalle sous une pression suffisante pour déplacer localement ladite première matière de revêtement liquide dans la couche de revêtement humide déjà sur ladite surface principale, pour établir ainsi une raie (344) de la seconde matière liquide de revêtement dans la couche de revêtement (12).

10. Procédé selon la revendication 9, caractérisé en ce que lesdites première et autre matières de revêtement sont pigmentées et diffèrent l'une de l'autre par le degré de pigmentation, de sorte que ladite raie est susceptible de distinction visuelle des parties de ladite couche de revêtement constituées par ladite première matière de revêtement.

11. Procédé selon la revendication 9 ou 10, également caractérisé par le stade consistant à mouvoir sélectivement une partie de ladite paroi de longueur étendue au-delà de ladite première ouverture, dans une direction parallèle à ladite surface principale et transversale au sens de l'avancement du feuillard pendant la progression du feuillard et la distribution de ladite autre matière de revêtement par ladite première ouverture, pour effectuer le mélange desdites première et autre matières de revêtement dans la raie et en position adjacente à celle-ci.

12. Procédé selon la revendication 11, caractérisé en ce que ladite paroi (26) est plane et comporte une partie mobile comprenant un disque (348) rotatif autour d'un axe perpendiculaire au plan de la paroi et en ce que le stade de mouvement consiste à effectuer un mouvement annulaire dudit disque autour dudit axe.

13. Procédé selon la revendication 9, également caractérisé en ce que le stade de déplacement de ladite première ouverture (336a) dans une direction parallèle à ladite surface principale et transversale à la direction de la progression du feuillard, pendant l'avancement du feuillard et la distribution de ladite autre matière de revêtement par ladite ouverture, pour changer progressivement l'emplacement de ladite raie (344b) le long dudit feuillard par rapport aux côtés dudit feuillard.

14. Procédé selon la revendication 13, caractérisé en ce que ladite paroi (26) de longueur étendue est plane et comprend une partie mobile comprenant un disque (352) rotatif autour d'un axe perpendiculaire au plan de la paroi, ladite première ouverture étant disposée dans ledit disque, et en ce que le stade de déplacement consiste à effectuer un mouvement angulaire dudit disque autour dudit axe.

15. Procédé selon la revendication 9, caractérisé en ce que ladite autre matière liquide de revêtement est distribuée audit intervalle sous pression comme stipulé à travers une série d'ouvertures (336a) espacées dans ladite paroi transversalement au sens de la progression du feuillard, pour ainsi établir une série correspondante de raies de cette autre matière liquide de revêtement dans ladite couche de revêtement.

16. Procédé selon la revendication 15, également caractérisé en ce qu'il comprend un stade consistant à déplacer progressivement lesdites ouvertures parallèlement à ladite surface principale et transversalement au sens de la progression du feuillard, pendant l'avancement du feuillard et la distribution de ladite autre matière de revêtement, pour varier progressivement les emplacements des raies dans le sens de la longueur du feuillard par rapport aux parois du feuillard.

17. Procédé selon la revendication 16, caractérisé en ce que le stade de mouvement de l'ouverture comprend le déplacement des ouvertures pour faire varier progressivement l'espacement entre les raies.

18. Procédé selon la revendication 17, caractérisé en ce que ladite paroi (26) de longueur étendue est plane et comprend une partie mobile comportant un disque rotatif autour d'un axe perpendiculaire à ladite surface principale, lesdites ouvertures étant disposées dans ledit disque, et le stade de déplacement des ouvertures consiste à déplacer angulairement ledit disque autour dudit axe.

19. Procédé selon la revendication 18, caractérisé en ce que lesdites ouvertures sont alignées en plusieurs rangées (438) excentrées par rapport audit axe, au moins l'une desdites rangées étant orientée suivant un angle aigu par rapport à au moins une autre desdites rangées.

20. Appareil pour former une couche de revêtement adhérent continu (12) sur une surface principale (10) d'un feuillard (11) de longueur indéterminée, comprenant des moyens définissant un trajet de progression (46) dudit feuillard longitudinalement par rapport à.lui-même, comportant une paroi étendue (26) en regard de ladite surface principale dudit feuillard et agencé de façon que le feuillard en progression se déplace longitudinalement par rapport à lui et des moyens (20; 122) pour empêcher uniformément ledit articule à l'encontre d'un mouvement de ladite surface principale (10) à l'écart de ladite paroi au-delà d'une distance prédéterminée pendant la progression dudit feuillard en regard de ladite paroi, des moyens formant un barrage (32) s'étendant transversalement par rapport au trajet de l'avancement du feuillard de manière à être disposés en . position adjacente mais espacés de la surface principale du feuillard et des moyens (22) pour fournir une matière de revêtement coulable à l'état humide à ladite surface principale devant ledit barrage, caractérisé en ce que ladite paroi étendue (26) est constituée par une surface d'un organe rigide (18; 120) surface qui est équidistante d'un support rigide constituant lesdits moyens d'empêchement et en ce que des moyens (42) sont prévus pour assujettir à demeure ledit organe rigide (18; 120) par rapport auxdits moyens d'empêchement.

21. Appareil selon la revendication 20, caractérisé en ce que l'extrémité de ladite paroi étendue éloignée de ladite première extrémité est formée comme une arête vive (47) pour empêcher la cavitation de la matière de revêtement humide sur ladite surface principale progressant au-delà de ladite paroi.

22. Appareil selon la revendication 20 ou 21, caractérisé en ce que le barrage (32) à ladite première extrémité de ladite paroi présente une surface s'approchant graduellement et progressivement de ladite paroi dans le sens de progression du feuillard.

23. Appareil selon l'une quelconque des revendications 20 à 22, caractérisé en ce que lesdits organes sont sous forme de plaques (18, 20) et en ce qu'une partie de la surface de l'une desdites plaques à l'extrémité d'entrée de l'espace entre les plaques constitue ledit barrage.

24. Appareil selon la revendication 23, caractérisé en ce que lesdits moyens d'assujettissement (42) sont réglables pour faire varier l'espacement entre lesdites surfaces en regard desdites plaques.

25. Appareil selon l'une quelconque des revendications 20 à 24, caractérisé en ce que les moyens de fourniture de la matière de revêtement comprennent des moyens pour débiter au moins deux compositions différentes de matières de revêtement à des parties différentes de ladite surface principale devant ledit barrage.

26. Appareil selon l'une quelconque des revendications 20 à 22, caractérisé en ce que lesdits moyens d'empêchement comprennent une surface sans fin mobile dans la même direction et à la même vitesse que le feuillard progressant dans ledit trajet.

27. Appareil selon la revendication 26, caractérisé en ce que lesdits moyens d'empêchement comprennent un rouleau (122) monté en rotation ayant une périphérie cylindrique qui constitue ladite surface sans fin et en ce que ladite paroi (128) est incurvée en conformité avec la périphérie du rouleau.

28. Appareil selon la revendication 27, caractérisé en ce que ledit rouleau (122) est monté en rotation autour d'un axe parallèle au barrage (136) et sensiblement dans un plan horizontal commun avec celui-ci et en ce que ladite paroi (128) est horizontalement mobile vers et depuis ledit rouleau (122).

29. Appareil selon l'une quelconque des revendications 20 à 28, caractérisé en ce que lesdits moyens de distribution comprennent des moyens pour établir et maintenir un réservoir enfermé de matière de revêtement coulable à l'état humide devant ledit barrage et en contact avec lui.

30. Appareil selon la revendication 29, également caractérisé par des moyens (230) pour varier la longueur dudit réservoir dans une direction transversale au feuillard.

31. Appareil selon la revendication 29 ou 30, caractérisé en ce que ledit réservoir est sous forme d'une tranchée allongée (184) s'ouvrant vers ladite surface principale du feuillard suivant la longueur dudit barrage et par ailleurs entièrement enfermée, et en ce que des moyens (202a) sont prévus pour fournir ladite matière de revêtement sous une pression positive à ladite tranchée (184) pour maintenir ladite tranchée entièrement remplie avec cette matière.

32. Appareil selon l'une quelconque des revendications 20 à 24, caractérisé en outre par des moyens pour débiter, à travers au moins une ouverture dans ladite paroi, vers au moins un emplacement dans ledit intervalle, une autre matière de revêtement liquide, sous une pression suffisante pour refouler localement la première matière de revêtement liquide dans la couche de revêtement, pour établir ainsi une raie (344) de ladite autre matière de revêtement liquide dans la couche de revêtement (12).

33. Appareil selon la revendication 32, caractérisé en ce que ladite paroi étendue est plane et présente une partie formée d'un disque (452) ayant une surface dans le même plan que ladite paroi et en ce qu'une série desdites ouvertures s'ouvrent à travers ladite surface du disque en des emplacements espacés, ledit disque étant monté en rotation autour d'un axe perpendiculaire à ladite paroi, des moyens étant prévus pour fournir ladite autre matière de revêtement liquide sous pression à travers lesdites ouvertures.

34. Appareil selon la revendication 33, caractérisé en ce que lesdites ouvertures (436) sont en alignement en au moins une rangée excentrée par rapport audit axe.

35. Appareil selon la revendication 33 ou 34, caractérisé en ce que la structure ayant une surface plane étendue constituant une partie fixe de ladite paroi étendue (26), et avec un bord transversal constituant ladite barrière, présente .en évidement circujaire (454) dans lequel est logé ledit disque, ce disque étant fabriqué en un matériau magnétique, et en ce qu'on prévoit un moyen de butée (470) débouchant dans ledit revêtement pour venir porter dans ledit disque et monter de façon réglable dans ladite structure en vue d'un mouvement dans une direction perpendiculaire au plan de ladite paroi (26) afin de positionner la surface dudit disque en rapport dans le même plan à ladite partie fixe de la paroi, et des moyens d'aimantation (472) montés dans ladite structure pour attirer ledit disque vers une position de contact avec ledit moyen de butée.

36. Appareil selon la revendication 32, caractérisé en ce que ladite paroi présente une gorge (362) s'étendant depuis ladite ouverture sensiblement dans le sens d'avancement dudit feuillard.
